



US007018946B2

(12) **United States Patent**  
**Shoemaker**

(10) **Patent No.:** **US 7,018,946 B2**  
(45) **Date of Patent:** **\*Mar. 28, 2006**

(54) **FABRIC INCLUDING POLYMER FILAMENTS HAVING PROFILED CROSS-SECTION**

(75) Inventor: **Richard T. Shoemaker**, Hixson, TN (US)

(73) Assignee: **Invista North America S.a.R.l.**, Wilmington, DE (US)

(\*) Notice: Subject to any disclaimer, the term of this patent is extended or adjusted under 35 U.S.C. 154(b) by 0 days.

This patent is subject to a terminal disclaimer.

(21) Appl. No.: **10/882,578**

(22) Filed: **Jul. 1, 2004**

(65) **Prior Publication Data**

US 2004/0242101 A1 Dec. 2, 2004

**Related U.S. Application Data**

(62) Division of application No. 10/367,236, filed on Feb. 14, 2003, now Pat. No. 6,884,505.

(51) **Int. Cl.**

**D01F 6/00** (2006.01)

(52) **U.S. Cl.** ..... 442/118; 442/192; 442/309; 428/357

(58) **Field of Classification Search** ..... 428/397, 428/357; 442/309, 192, 118

See application file for complete search history.

(56) **References Cited**

**U.S. PATENT DOCUMENTS**

2,959,839 A 11/1960 Craig

|                 |         |                         |
|-----------------|---------|-------------------------|
| 3,416,952 A     | 12/1968 | McIntyre et al.         |
| RE29,363 E      | 8/1977  | McKay                   |
| 4,083,914 A     | 4/1978  | Schippers et al.        |
| 4,239,720 A     | 12/1980 | Gerlach et al.          |
| 4,408,977 A     | 10/1983 | Phillips                |
| 4,468,505 A     | 8/1984  | Bowen et al.            |
| 4,472,477 A     | 9/1984  | Phillips                |
| 5,057,368 A     | 10/1991 | Largman et al.          |
| 5,108,838 A     | 4/1992  | Tung                    |
| 5,152,014 A     | 10/1992 | Marx et al.             |
| 5,168,143 A     | 12/1992 | Kobsa et al.            |
| 5,176,926 A     | 1/1993  | Tung                    |
| 5,208,106 A     | 5/1993  | Tung                    |
| 5,447,771 A     | 9/1995  | Mills et al.            |
| 6,884,505 B1 *  | 4/2005  | Shoemaker ..... 428/364 |
| 2002/0034903 A1 | 3/2002  | Shoemaker et al.        |

**FOREIGN PATENT DOCUMENTS**

|    |             |        |
|----|-------------|--------|
| CA | 1 234 656   | 4/1988 |
| GB | 1 233 585 A | 5/1971 |
| JP | 64-20243    | 7/1987 |

\* cited by examiner

*Primary Examiner*—N. Edwards

(74) *Attorney, Agent, or Firm*—Robert B. Furr, Jr.

(57) **ABSTRACT**

The present invention is directed to a multi-filament yarn formed at least in part from filaments having cross-sectional zig-zag or double "W" shape with a 180 degree axis of symmetry. The filaments have a denier per filament generally in the range of about 0.1 to about 4.0. Fabrics made from yarns formed with the filaments have high moisture wicking, soft hand, and a silk-like lustrous appearance.

**9 Claims, 2 Drawing Sheets**





Figure 5



## 1

**FABRIC INCLUDING POLYMER  
FILAMENTS HAVING PROFILED  
CROSS-SECTION**

**CROSS-REFERENCE TO RELATED  
APPLICATIONS**

The present patent application is a division of U.S. patent application Ser. No. 10/367,236 filed on Feb. 14, 2003 in the name of Richard T. Shoemaker now U.S. Pat. No. 6,884,505. 10

**FIELD OF THE INVENTION**

This invention relates to synthetic polymer filaments having a double "W" profiled cross section normal to the longitudinal axis of the filament and a 180 degree axis of symmetry. 15

**BACKGROUND OF THE INVENTION**

Textile fibers or filaments from synthetic polymers, particularly polyamide polymers like nylon 66 and nylon 6, and multi-filament yarns melt-extruded from the same polyamide polymers, are produced for many apparel uses. The most common cross-sectional (taken longitudinally to the long axis of the filament) shape for each filament comprising the multi-filament yarns is circular. However, many variations on the individual filament cross-sectional shapes exist. These include a "dogbone" cross-sectioned filament commercially available from E. I. DuPont de Nemours and Company of Wilmington, Del. USA and known as TAC-TEL® Diabolo. A bi-lobal filament cross-sectional shape is disclosed in U.S. Patent Application Number 2002-0034903-A1 (Shoemaker, et al.). Other known shapes include tri-lobed or even 6-lobed, disclosed in Japanese Kokoku patent document 01-20243 (Nihon Ester KK). Another multi-lobal cross-sectioned fiber, available from DuPont and known as Coolmax™, is shown in U.S. Pat. No. 5,152,014.

Filaments with cross-sectional shapes other than circular provide multi-filament yarns for fabrics and garments with varied visual aesthetics including those known in the art as glitter, sparkle, matt appearance, and increased opacity or cover. Lighter fabric weight and fabric flatness are also achieved through variations in the individual filament cross-sectional shape. Among these numerous profiled cross section fibers used in synthetic filaments for apparel, certain other cross sections have been developed to enhance the ability of filaments to absorb or wick moisture.

Moisture wicking, which refers to the capillary movement of water through or along the fibers, is considered a desirable feature in apparel fabrics as it improves comfort to the wearer by spreading moisture away from the skin so that it can evaporate more readily. In addition, combinations of cross-sections, denier per filament (dpf), and finish preparations applied to filaments and fabrics have been developed to enhance the ability of filaments to absorb or wick moisture. For example, "two-sided" fabrics have been developed to help move moisture from the inside to the outside of the fabric due to the surface chemistry. Typically, the two-sided fabrics have fine denier per filament (dpf) filaments primarily on the outside, and coarser dpf filaments primarily on the inside. Although this "two-sided" fabric is readily accomplished in weft knit fabrics through knitting construction, there is room for further improvement in wicking through optimum shape of the individual filaments. In addition, warp knit and woven fabrics are difficult and

## 2

expensive to construct in a manner to maintain filament location primarily on one side or the other. Therefore, especially in woven and warp knits, a filament that provides superior moisture wicking is needed to improve wearer comfort, especially for active wear. 5

There is a continuing need to provide multifilament synthetic yarns that provide enhanced moisture wicking properties to fabrics as well as a soft fabric hand and silk-like luster for apparel.

**SUMMARY OF THE INVENTION**

The present invention relates to a multi-filament yarn formed at least in part from synthetic polymer filaments having double "W" transverse cross-sectional shapes (as viewed normal to the longitudinal axis of the filaments). 15

In the preferred embodiment the filament transverse cross-section includes at least seven contiguous segments in zig-zag configuration. Preferably, adjacent segments form 20 an angle between about 40 degrees and about 60 degrees. The filament cross-section has a nominal width, a nominal length and a nominal thickness. The ratio of the nominal width to the nominal thickness preferably is less than about 3, and the indentation to thickness ratio preferably is 25 between about 0.25 and 0.6. Preferably, the filament has a denier per filament between about 0.1 and about 4.0.

Preferably, the synthetic polymer filament comprises a polyamide synthetic polymer selected from the group consisting of: polyhexamethylene adipamide; polycaproamide; 30 polyanthamide; nylon 10; polydodecanolactam; polytetramethylene adipamide; polyhexamethylene sebacamide homopolymer; a polyamide of n-dodecanedioic acid and hexamethylenediamine homopolymer; and a polyamide of dodecamethylenediamine and n-dodecanedioic acid.

35 A yarn may be formed at least in part from the synthetic polymer filament of the invention. Where the yarn is formed from a number of filaments, the synthetic polymer filament of the invention preferably comprises at least about 50% of the total number of filaments in said yarn. Preferably the yarn has a denier between about 15 and about 200.

40 A fabric may be formed with the yarn that includes synthetic polymer filaments according to the invention. A double-sided fabric may include the yarns that include the fibers or the fibers according to the invention on one side or both sides. A wetting agent may be applied to one side of the fabric to enhance moisture wicking. Suitable wetting agents include hydrophilic polyamide, hydrophilic silicone, and hydrophilic polyester.

45 The synthetic polymer filament according to the invention preferably has a transverse cross-section that includes seven contiguous segments in zig-zag configuration, wherein each segment defines a proximal end and a distal end, wherein a distal end of a first segment is connected to a proximal end of a second segment, wherein a distal end of the second segment is connected to a proximal end of a third segment, wherein a distal end of the third segment is connected to a proximal end of a fourth segment, wherein a distal end of the fourth segment is connected to a proximal end of a fifth segment, wherein a distal end of the fifth segment is connected to a proximal end of a sixth segment, wherein a distal end of the sixth segment is connected to a proximal end of a seventh segment, and wherein a pivot point is defined along the fourth segment and the transverse cross-section of the filament is symmetrical when rotated 180 degrees about 50 said pivot point. In this zig-zag transverse cross-section configuration, the adjacent segments preferably form an angle between about 40 degrees and about 60 degrees. A 55

yarn may be formed at least in part from the synthetic polymer filament with the zig-zag transverse cross-section configuration, and a fabric may be constructed from such yarn or filaments. The fabric may be a double-sided fabric to which a wetting agent has been applied to one side to enhance moisture wicking.

The filaments according to the present invention are especially suitable in making apparel fabrics having a high moisture-wicking capability, combined with a soft hand and a silk-like lustrous appearance.

#### BRIEF DESCRIPTION OF THE DRAWINGS

FIG. 1 is a representation of a filament according to the invention having a double "W" transverse cross-sectional shape;

FIG. 2 is a representation of a spinneret plate having four capillaries each comprising 7 slots for making filaments according to the invention having a double "W" transverse cross-sectional shape;

FIG. 3 is a representation of a single spinneret capillary comprising seven slots for making filaments having a double "W" transverse cross-sectional shape;

FIG. 4 is a representation of a cross-section of a preferred embodiment of the double-W cross-sectionally shaped filament according to the invention; and

FIG. 5 is a representation of a yarn formed from a combination of filaments including filaments with the double "W" transverse cross section.

#### DETAILED DESCRIPTION OF THE INVENTION

The transverse cross-sectional shape of the filaments of the invention is a double "W" shape having a 180 degree axis of symmetry as represented in FIG. 1. The double "W" shape includes an upright "W" sharing a fourth leg with an inverted "W". The 180 degree axis of symmetry means that when the cross-section is rotated 180 degrees about its center point P, the rotated cross-sectional shape is identical to the initial cross-sectional shape prior to rotation. The center point P shown in FIG. 1 is for reference in this description and would not be visible in this manner on a filament according to the invention.

The preferred filament transverse cross-sectional shape is comprised of seven contiguous segments originating from a first free end 1a of the cross-sectional shape and traversing through the seven segments (10, 20, 30, 40, 50, 60 and 70) to free end 7 of the seventh segment 70. The first segment 10 connects to the second segment 20 at a first vertex 1b formed at the junction of the first segment 10 with the second segment 20. The second segment 20 connects to the third segment 30 at a second vertex 2 formed at the junction of the second segment 20 with the third segment 30. The third segment 30 connects to the fourth segment 40 at a third vertex 3 formed at the junction of the third segment 30 with the fourth segment 40. The fourth segment 40 connects to the fifth segment 50 at a fourth vertex 4 formed at the junction of the fourth segment 40 with the fifth segment 50. The fifth segment 50 connects to the sixth segment 60 at a fifth vertex 5 formed at the junction of the fifth segment 50 with the sixth segment 60. Finally, the sixth segment 60 connects to the seventh segment 70 at a sixth vertex 6 formed at the junction of the sixth segment 60 with the seventh segment 70. The cross-section terminates at second free end 7. In this configuration, the adjacent segments preferably form an angle between about 40 degrees and about 60 degrees.

The filaments of the invention are composed of a synthetic thermoplastic polymer. More particularly the filaments of the present invention may comprise of homopolymers and copolymers of melt-spinnable polymers. 5 Particularly preferred melt-spinnable polymers include polyamides, such as polyhexamethylene adipamide (nylon 6,6); polycaproamide (nylon 6); polyenanthamide (nylon 7); nylon 10; polydodecanolactam (nylon 12); polytetramethylene adipamide (nylon 4,6); polyhexamethylene sebacamide homopolymer (nylon 6,10); a polyamide of n-dodecanedioic acid and hexamethylenediamine homopolymer (nylon 6,12); and a polyamide of dodecamethylenediamine and n-dodecanedioic acid (nylon 12,12).

Methods of making the homopolymers and copolymers 15 used in the present invention are known in the art and may include the use of catalysts, co-catalysts, and chain-branchers to form the copolymers, as known in the art. Preferably, the fiber-forming polymer is at least one polyamide, since polyamides are generally softer due to the lower modulus, 20 and they are more hydrophilic due to their surface chemistry. More preferably, the polymer is a polyamide such as nylon 6, nylon 6,6, or a combination thereof. Most preferably, the polyamide is nylon 6,6.

The polymers and resultant filaments, yarns, and apparel 25 articles of the present invention can comprise conventional additives, which are added during the polymerization process or to the formed polymer or article, and may contribute towards improving the polymer or fiber properties. Examples of these additives include antistatics, antioxidants, 30 antimicrobials, flameproofing agents, dyestuffs, light stabilizers, polymerization catalysts and auxiliaries, adhesion promoters, delustrants, such as titanium dioxide, matting agents, organic phosphates, and combinations thereof.

The polymers and resultant filaments, yarns, fabrics and 35 apparel articles of the present invention can be treated on their surface with permanent or semi-permanent hydrophilic treatments or finishes. These treatments generally improve the moisture wicking property of the fabrics and apparel articles. Suitable surface treatments useful in the present 40 invention include hydrophilic polymeric compositions, such as polyamides made with hydrophilic segments, such as poly(hexamethylene adipamide)-poly[poly(oxyethylene) adipamide] copolymers [CAS No. 92717-79-8], such as described in U.S. Pat. No. 4,468,505 incorporated herein by 45 reference in its entirety; hydrophilizing silicone microemulsions, such as "Sandotol HV Liquid", which is commercially available from Clariant; hydrophilic copolymers, such as a copolyester containing both polyoxyethylene diester and alkylene diester segments; and certain nonionic 50 surfactants, such as those described in Canadian Patent No. 1,234,656. These surface treatments vary in their ability to improve water wicking performance and vary in their durability or resistance to removal by washing. This variability in performance depends on several factors, including the 55 composition of the treated fiber, the amount of wicking treatment applied to the fiber, and the resistance of the treatment to washing.

The poly(hexamethylene adipamide)-poly[poly(oxyethylene) adipamide] copolymers have been found to be particularly 60 useful to treat articles of the present invention. The polymers are composed of polyoxyethylene adipamide segments and poly(hexamethylene adipamide) segments. The poly(oxyethylene) adipamide segments are formed from the reaction of a poly(oxyethylene) diamine [CAS No. 65605- 65 36-9] with adipic acid. The poly(oxyethylene) diamine can include minor amounts, for example, less than 25 mol % oxypropylene groups with the oxyethylene groups.

The polyoxyethylene adipamide segments have high affinity for water and impart hydrophilic character to the copolymer and thus to the treated fiber, while the poly(hexamethylene adipamide) segments have low water solubility and thus impart permanence to the treatment on the fiber. These adipamide copolymers are especially useful when the polymer used in the substrate to be treated is nylon 6, nylon 6,6, or combinations thereof, and are most preferred for use when the polyamide is nylon 6,6.

The length of each of the polyoxyethylene adipamide and poly(hexamethylene adipamide) segments may be varied. Increasing the length of the polyoxyethylene adipamide segments increases the water wicking property of the treatment while simultaneously increasing its water solubility and thus decreasing its durability to washing. Increasing the length of the poly(hexamethylene adipamide) segments decreases its water solubility and thus increases its durability of the treatment to washing.

The suitable length of the polyoxyethylene adipamide segment is also determined to an extent by commercial availability of the poly(oxyethylene) diamine. Poly(oxyethylene) diamines with molecular weights of 600, 900, and 2000 are available from Huntsman Corporation, and hence are especially useful. They are known as XTJ-500, XTJ-501, and XTJ-502.

The relative amount of each of these segments to each other in the treatment composition may also be varied in any desired ratio. Increasing the proportion of polyoxyethylene adipamide segments increases the water wicking property of the treatment while simultaneously increasing its water solubility and thus decreasing its durability to washing. Conversely, increasing the proportion of the poly(hexamethylene adipamide) segments decreases its water solubility and thus increases its durability to washing. Balancing the relative amounts and lengths of the polyoxyethylene adipamide and poly(hexamethylene adipamide) segments in the copolymer can be done to maximize the water wicking performance while maintaining suitable durability to repeated washing. A preferred copolymer for the present invention employs poly(oxyethylene) diamines of molecular weight between about 900 and about 2000 with weight percentages of nylon 6—6 ranging from about 18–22%. The polymers can be made as described in U.S. Pat. No. 4,468,505.

These copolymers can be dissolved in any suitable solution when used in the present invention. A preferred system has been found to be a solution of 1,2-propanediol and water. This combination provides a solution that may be either applied to fabrics by itself or in combination with other processing agents as described below. The amount of poly(hexamethylene adipamide)-poly[poly(oxyethylene) adipamide] copolymer in the solution may range from about 0.1% to about 40% by weight. The most preferred range is from about 8% to about 15%. At higher percentages of copolymer, the solution has a tendency to gel. Lower percentages are acceptable, but are less economical. For application to fabric, the solution may be further diluted with water to facilitate the application of only the desired amount of finish without over-application. 1,2-propanediol is used to facilitate dissolution of the copolymers in water. A preferred amount of 1,2-propanediol is approximately equal in weight to the hydrophilic polyamide copolymer. More 1,2-propanediol may be used (e.g. 1.5 times the weight of copolymer), but may lengthen the drying time required in the application process. Less 1,2-propanediol may be used (e.g. 0.5 times the weight of copolymer), but reduces the solubility of the hydrophilic polyamide copolymer. The use of

1,2-propanediol is preferred over ethanol as taught in U.S. Pat. No. 4,468,505 because it is not flammable, it is less toxic, less carcinogenic, less of it may be used, and it has a higher boiling point and so is less fugitive.

5 Hydrophilic copolymers are also useful hydrophilic agents in the present invention. Hydrophilic copolymers include copolymers containing both polyoxyethylene diester and alkylene diester segments. They may be simple copolymers, i.e., they may contain only polyoxyethylene 10 diester and polyalkylene diester segments, the copolyester being derived from a single polyethylene oxide, diester and glycol. Polyethylene oxides of various molecular weights, dimethyl terephthalate, and ethylene glycol are the most 15 common raw materials for these copolymers, mainly because of cost and availability. Numerous variations on the comonomers used to prepare these simple hydrophilic copolymers are possible. These copolymers are disclosed in U.S. Pat. No. 3,416,952, incorporated herein by reference in its entirety. Examples of these copolymers include "ZEL- 20 CON" 5126 [CAS No. 9074-67-3], which is commercially available from Stepan Company, and "MILEASE" T [CAS No. 9016-88-0], which is commercially available from Imperial Chemical Industries, Limited, London, England. Both "ZELCON" 5126 and "MILEASE" T are sold in an 25 aqueous dispersion form containing up to 85% water.

These permanent or semi-permanent hydrophilic treatment compositions previously described may be applied to the fabric or fiber by any suitable means such as wiping, painting, dipping, foaming, feeding at the nip of a roller, spraying, or other means. The composition is typically 30 applied at a minimum level of at least 0.1% weight of solids on fiber, preferably at least 0.5% weight of solids on fiber, to achieve water wicking and durability. Application at higher levels will improve hydrophilic character. After drying or removal of the solvent, a durable hydrophilic coating remains on the fabric or fiber surface. This coating causes water placed on the surface to rapidly wet the fabric and to move along the fiber length and through the fabric layer.

Other additives that may be applied on the fibers, for 35 example, during spinning and/or drawing processes include antistatics,slickening agents, adhesion promoters, antioxidants, antimicrobials, flameproofing agents, lubricants, and combinations thereof. Moreover, such additional additives may be added during various steps of the process as is 40 known in the art.

45 Filaments of the present invention having the transverse double "W" cross-section can be mixed with filaments of other cross-sections, e.g. circular cross-section, and/or polymers to form yarns. FIG. 5 is a representation of a yarn 100 comprising a plurality of filaments with the transverse double "W" cross section 110 and filaments with a larger dpf 50 and varying cross section 120. The filaments 110 have indentations 80 along their longitudinal length which serve as channels to direct moisture.

55 The filaments of the present invention are formed by any suitable spinning method, which may vary based upon the type of polymer used, as is known in the art. Generally, the melt-spinnable polymer is melted and the molten polymer is extruded through a spinneret capillary orifice having a 60 design corresponding to the desired double "W" cross-section of the present invention. The extruded fibers are then quenched or solidified with a suitable medium, such as air, to remove the heat from the fibers leaving the capillary orifice. After quenching, the filaments are converged, interlaced, and wound as a multifilament bundle.

65 The spinneret capillary used to produce the filaments of the present invention can be any suitable capillary capable of

producing the transverse double "W" cross-section described above. One suitable spinneret capillary plate is represented by instant FIG. 2, which shows four rows of slot openings, with each row having seven slots spaced apart from one another and angled in a zig-zag configuration. The spinneret plate diagrammatically represented by FIG. 2 is capable of forming four (4) identical filaments of the transverse double "W" cross-sectional shape.

A single row of spinneret capillary slots is represented in FIG. 3. An angle  $\theta$  formed by any pair of adjacent slot segments is between about 40° and 600 degrees of arc. Moreover, referring to FIG. 3, the slot segments may have any length (L), for example, from about 0.130 mm to about 130 mm, preferably between about 0.25 mm to about 0.50 mm, and any width (D), such as between about 0.025 mm to about 0.40 mm, preferably about 0.075 mm to about 0.130 mm.

The spinneret capillaries through which the molten polymer is extruded, represented by FIG. 3, are cut to produce the desired cross-section of the present invention. The capillaries or spinneret bore holes may be cut by any suitable method, such as by laser cutting, as described in U.S. Pat. No. 5,168,143, herein incorporated by reference, drilling, Electric Discharge Machining (EDM), and punching, as is known in the art. Preferably, the capillary orifice is cut using a laser beam.

The dimensions for filaments of the preferred embodiment are further defined with reference to a filament 110 shown in FIG. 4. In FIG. 4, the width (A), the maximum thickness (B) and the minimum thickness (b) of the cross section of the spun filaments are represented. As shown in FIG. 4, the filament cross-section is shaped such that indentations 80 are disposed opposite each vertex. The maximum thickness (B) is measured as the distance between two sequential vertexes (such as 1b and 2), while the minimum thickness (b) is measured as the distance between two sequential indentations 80. The indentation-to-thickness ratio (ITR) of the filament cross-section, which is important in determining the moisture wicking ability of the filament, is given by the equation  $ITR=1-b/B$ .

Preferably, the filaments according to the invention have a cross-sectional width (A) ranging between about 28 and 42 microns, and most preferably between about 28 and 35 microns. Preferably, for filaments having a denier per filament of about 3, the maximum thickness (B) is between about 12 and 15 microns, and the minimum thickness (b) is between about 5 and 10 microns. The preferred spun filament has a ratio of A/B of less than 3, and an indentation to thickness ratio (ITR) of between about 0.25 and 0.60. Most preferably, the ITR is between about 0.40 and 0.60, which indicates that the indentations 80 (FIG. 4) are deeper and will provide superior moisture movement along the length of the filament.

The filaments can be formed into any type of yarn, for example, fully drawn yarns or partially oriented yarn, as used, for example, in texturing feed yarns. Accordingly, in one embodiment, the filaments are spun as a fully drawn yarn, for example, a yarn having an orientation of about 35 to about 50% elongation to break, which may be immediately used in manufacturing fabrics and apparel articles. Optionally, however, the filaments of the present invention may be textured, also known as "bulked" or "crimped," according to known methods. In this embodiment of the invention, the filaments may be drawn as a partially oriented yarn, for example, a yarn having an orientation of about 55 to about 75% elongation to break, and then textured by

techniques, such as by draw false-twist texturing, air-jet texturing, gear-crimping, and the like.

The filaments of the invention can be processed into a multifilament fiber or yarn having any desired denier, filament count, and denier per filament (dpf). The yarn formed from the filaments of the present invention typically has a total denier between about 10 and about 300 denier, preferably, between about 15 and about 250 denier, and most preferably, between about 20 and about 150 denier. The filaments of the present invention also typically have a denier per filament between about 0.1 to about 4 dpf, preferably, between about 0.8 to about 3.5, and most preferably, between about 0.9 to about 3.0. In one embodiment, the dpf is less than about 2.9, or less than about 2.5. The double "W" cross-section filaments can be mixed with other filaments, for example, having a dpf above or below about 4.

The yarns of the present invention may further be formed from a plurality of different filaments having different dpf ranges. In such case, the yarns should be formed from at least one filament having the multilobal cross-section of the present invention. Preferably, each filament of a yarn containing a plurality of different filaments has the same or different dpf, and each dpf is between about 0.1 to about 4 dpf, preferably, between about 0.8 to about 3.5, and most preferably, between about 0.9 to about 3.0.

The filaments of the present invention may be used to make fabrics. Any known suitable method of making fabrics may be used. For example, warp knitting, circular knitting, hosiery knitting, and laying a staple product into a non-woven fabric are suitable for making fabrics. In one embodiment, two-sided fabrics are made using the filaments of the present invention on primarily one side of the fabric. Any other type of yarn may be used to make up the other side of the fabric, but preferably such other yarn has a different wicking ability. Suitable yarns for the other side of the two-sided fabric may be made up of polyamides, polyesters, polyolefins, natural fibers, such as cotton, wool, silk, rayon, and combinations thereof. The two-sided fabrics may be made by methods known in the art. For example, the fabrics may be knitted using the multifilament yarn having double "W" cross-sections of the present invention on one side and another yarn on the other side. Suitable methods of making the two-sided fabrics include warp knitting and plating the yarns. The two-sided fabrics have the benefit of allowing moisture to be drawn away from the body. Generally, the higher dpf fabric is used on the inside of a garment, and the lower dpf fabric is used on the outside of the garment. However, the double "W" cross-section multifilament yarns of the present invention may be used on either side of the two-sided fabric. For example, the double "W" cross-section multi-filament yarns of the present invention may be used on the outside of the fabric and treated with a finishing agent, such as a hydrophilic agent as described above. In another embodiment, a different yarn, such as cotton, may be used to form the outside of the fabric with the double "W" multi-filament yarns on the inside.

In another preferred embodiment, the yarn is formed from at least about 50%, preferably at least about 80%, of the filaments of the present invention based on the total number of filaments, and such yarn is processed into a fabric. In yet another preferred embodiment, the yarn or fabric formed from the filaments of the present invention is combined with a permanent or semi-permanent hydrophilic wetting agent as described above. The fabrics are useful to make any type of apparel article, including swimwear, active wear, and ready-to-wear garments.

Any desired additional agent may be applied directly to the fabrics. Examples of these additives include antistatics, antioxidants, antimicrobials, flameproofing agents, dye-stuffs, light stabilizers, polymerization catalysts and auxiliaries, adhesion promoters, delustrants, such as titanium dioxide, matting agents, organic phosphates, permanent or semi-permanent hydrophilic wetting agent, and combinations thereof. Preferably, a suitable wetting agent is added to fabrics made using the multifilament yarns of the present invention. Suitable wetting agents for application directly to the fabric include hydrophilic agents, as described above.

The fabrics made using the filaments and yarns of the present invention have been found to exhibit excellent moisture wicking properties, soft hand, and silk-like high luster. The moisture wicking of the yarns of the invention is determined by known methods, such as by a vertical wicking test or a horizontal wicking test. The vertical wicking test may be conducted by knitting the yarns into tubes, and then either scouring or treating the tubes with any desired agent and allowing the treated tubes to air dry. The tubes are then cut into 1 inch (25.4) wide strips about 8 inches (203 mm) long and suspended vertically above water with 3 inches (75 mm) in the water and 5 inches (125 mm) above the water. Observations of the height of the water being wicked up the strips are conducted visually at predetermined times, such as at 1 minute, 5 minutes, 10 minutes, 20 minutes and 30 minutes.

The yarns of the present invention have a tenacity suitable for use in apparel. Tenacity is measured on an Instron equipped with two grips which hold the yarns at the gauge lengths of 10 inches. The yarn is then pulled by the strain rate of 10 inch/minute, the data are recorded by a load cell, and stress-strain curves are obtained. Tenacity is the breaking strength (in grams) divided by the yarn's denier. Both partially oriented yarns and fully drawn yarns of the present invention can have a tenacity of between about 2 to about 8, preferably between about 3 to about 6 grams per denier.

The elongation-to-break of the yarn can be measured using any known apparatus. For example, one method involves pulling to break on an Instron Tester TTB (Instron Engineering Corporation) with a Twister Head made by the Alfred Suter Company and using 1-inch×1-inch (25 mm×25 mm) flat-faced jaw clamps (Instron Engineering Corporation). Samples typically about 10-inches in length are subjected to two turns of twist per inch at a 60% per minute rate of extension at 65% Relative Humidity and 70° F. (21° C.). The elongation to break for both fully drawn yarns and partially oriented yarns of the present invention was between about 30% to about 80%, preferably between about 40% to about 60%.

The boil off shrinkages of the yarn may be measured using any known method. For example, it may be measured by suspending a weight from a length of yarn to produce a 0.1 gram/denier load on the yarn and measuring its length ( $L_0$ ). The weight is then removed and the yarn is immersed in boiling water for 30 minutes. The yarn is then removed, loaded again with the same weight, and its new length recorded ( $L_f$ ). The percent shrinkage (S) is calculated by using the formula:

$$\text{Shrinkage (\%)} = 100 \frac{(L_0 - L_f)}{L_0}$$

A low shrinkage is highly desirable for most textile purposes. The yarns of the present invention have a shrinkage less than about 10%, preferably less than about 7%, most preferably less than about 6%.

The invention will now be illustrated by the following non-limiting examples.

## EXAMPLES

## Example A

- 5 An 80 denier-26 filaments double "W" transverse cross-section yarn was spun at a temperature of 290° C. The yarn was spun with nylon 6,6, having a relative viscosity (RV) of between 45–47. A normal nylon pack formulation was used using spinnerets in a configuration of three ends per pack 10 having the double "W" transverse cross-section. The nylon 6,6 was spun at a windup speed of 3000–3200 yards per minute and drawn at a draw ratio of 2.5–2.7×. The tenacity of the filaments was 3.6 grams per denier, and the yarn had an elongation to break of 42%. The yarn had a cross-section 15 shape of substantially that presented in FIG. 4. Normal spin/secondary spin finishes were used. A photomicrograph of the yarn is shown in FIG. 5.

The yarn was woven in a six harness irregular satin weave. After weaving, each sample was tested via a vertical wicking test. The samples were scoured thoroughly to remove all finishes. The sample was cut into 1 inch (25 mm) wide strips about 8 inches long and then suspended vertically above the water with three (3) inches (75 mm) in the water and five (5) inches (125 mm) above the water. The 20 height of water wicking up the strip, up to five (5) inches (125 mm), was measured as a function of time. Observations were made at 1 minute, 5 minutes, 10 minutes, and 30 minutes. The test was stopped when five (5) inches (125 mm) was reached.

## Comparative Examples 1 and 2

Control cross-sections were also measured for comparison. These control yarns were of bilobal (also known as "silkworm") and dogbone (also known as "diabolo") cross-sections, and each was formed of the same nylon 6,6 polymer. A silkworm cross-section filament yarn of 80 denier and 28 filaments (Example a) and a diabolo cross-section filament yarn of 90 denier and 26 filaments (Example 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 970

## 11

While the invention has been described in connection with preferred embodiments, variations within the scope of the invention will likely occur to those skilled in the art. Thus, it is understood that the invention is covered by the following claims.

What is claimed is:

1. A fabric formed from a yarn comprising at least in part a synthetic polymer filament, wherein said filament comprises a transverse cross-section that includes seven contiguous segments in zig-zag configuration, wherein each segment defines a proximal end and a distal end, wherein a distal end of a first segment is connected to a proximal end of a second segment, wherein a distal end of the second segment is connected to a proximal end of a third segment, wherein a distal end of the third segment is connected to a proximal end of a fourth segment, wherein a distal end of the fourth segment is connected to a proximal end of a fifth segment, wherein a distal end of the fifth segment is connected to a proximal end of a sixth segment, wherein a distal end of the sixth segment is connected to a proximal end of a seventh segment, and wherein a pivot point is defined along the fourth segment and the transverse cross-section of the filament is symmetrical when rotated 180 degrees about said pivot point; and wherein said fabric is a double sided fabric comprising said synthetic polymer filament on one side of said fabric; and further wherein a wetting agent is applied to the one side of said fabric.

2. The fabric of claim 1 wherein adjacent segments of the synthetic polymer filament form an angle between about 40 degrees and about 60 degrees.

3. The fabric of claim 1, wherein the synthetic polymer filament comprises a polyamide synthetic polymer selected

## 12

from the group consisting of: polyhexamethylene adipamide; polycaproamide; polyenanthamide; nylon 10; polydodecanolactam; polytetramethylene adipamide; polyhexamethylene sebacamide homopolymer; a polyamide of n-dodecanedioic acid and hexamethylenediamine homopolymer; and a polyamide of dodecamethylene diamine and n-dodecanedioic acid.

4. The fabric of claim 1 wherein the synthetic polymer filament has a denier per filament of about 1.0 to about 4.0.

5. The fabric of claim 1 wherein the synthetic polymer filament has an indentation-to-thickness ratio between about 0.25 and about 0.6.

6. The fabric of claim 1, wherein the yarn comprises at least about 50% of the total number of filaments in said yarn of the synthetic polymer filaments.

7. The fabric of claim 1 wherein the yarn formed from the synthetic polymer filaments has a denier between about 15 and about 200.

8. The fabric of claim 1, wherein said wetting agent is selected from the group consisting of a hydrophilic polyamide, hydrophilic silicone, and hydrophilic polyester.

9. A fabric comprising at least in part a synthetic polymer filament having a transverse cross-section having multiple segments arranged in a double "W" shape including a upright W-shaped portion sharing a segment with an inverted W-shaped portion, wherein said fabric is double-sided fabric comprising said synthetic polymer filament on one side of said fabric; and further wherein a wetting agent is applied to the one side of said fabric.

\* \* \* \* \*

UNITED STATES PATENT AND TRADEMARK OFFICE  
**CERTIFICATE OF CORRECTION**

PATENT NO. : 7,018,946 B2  
APPLICATION NO. : 10/882578  
DATED : March 28, 2006  
INVENTOR(S) : Richard T. Shoemaker

Page 1 of 1

It is certified that error appears in the above-identified patent and that said Letters Patent is hereby corrected as shown below:

Title Page, Item [73] under Assignee, delete "Invista North America S.a.R.L." and replace it with -- INVISTA North America S.à r.l. --

At page 10, Claim 1, at line 17, delete "filth" and replace it with -- fifth --.

Signed and Sealed this

Twenty-second Day of August, 2006

A handwritten signature in black ink, appearing to read "Jon W. Dudas". The signature is written in a cursive style with a large, stylized "J" and "W".

JON W. DUDAS  
*Director of the United States Patent and Trademark Office*